

July 9, 1929.

F. C. LANGENBERG

1,720,366

METHOD OF MAKING HOLLOW METALLIC ARTICLES

Filed Dec. 11, 1925



Fig. 1.



Fig. 2.



Fig. 3.



Fig. 4.



Fig. 5.



Fig. 6.



Fig. 7.



Fig. 8.

INVENTOR:

Frederick C. Langenberg  
By MacLeod Kahn, Lyman & Wake,  
Atty's.

Patented July 9, 1929.

1,720,366

# UNITED STATES PATENT OFFICE.

FREDERICK C. LANGENBERG, OF WATERTOWN, MASSACHUSETTS, ASSIGNOR OF ONE-HALF TO TRACY C. DICKSON, OF WATERTOWN, MASSACHUSETTS.

## METHOD OF MAKING HOLLOW METALLIC ARTICLES.

Application filed December 11, 1925. Serial No. 74,816.

My present invention relates to a novel method of manufacturing hollow metallic articles and particularly those made of steel. In my prior Patent No. 1,553,824, September 15, 1925, I have described a method for making metallic articles which consists essentially in expanding the article to a point beyond the elastic limit of the material employed while it is contained within a jacket which 10 stops the expansion when a predetermined point has been reached. In another prior Patent No. 1,552,848, September 8, 1925, I have described another method which includes annealing the material after the first 15 expansion and then again expanding it to a point beyond its elastic limit. As explained in this patent, the strength of the article produced is increased by interposing the annealing step between the expanding 20 steps.

I have discovered that when a unitary cylinder is expanded beyond the elastic limit of the metal composing it, the elastic limit of the metal at the bore will be raised to a 25 greater extent than that of the metal at the outside of the cylinder. Consequently the total elastic strength of the article, that is, the total ability of the article to resist an internal pressure without permanent distortion is not as great as it would be if the 30 elastic limit of the metal in the outer parts of the structure had been distributed in a different manner.

My improved process makes it possible to 35 produce a hollow cold-worked article, the elastic limit to whose exterior layer of metal is not greatly different from that of its interior layers, so that the total strength of an article of a given weight and material is 40 much increased.

The herein-described novel method therefore produces composite articles which are stronger for a given weight and material, or are lighter for a given strength than articles 45 made of a single piece of metal as described in my said prior patents.

The herein-described novel method is particularly applicable to the manufacture of large guns and similar articles and does 50 away with the expensive, difficult and unreliable methods of shrinking on successive rings which have heretofore been commonly employed in the manufacture of guns. The compound guns manufactured by the herein-described improved method have an elastic

strength materially greater than either a one-piece gun made by the methods described in my two prior patents above mentioned, or of a built-up gun made by the ordinary method of shrinking on rings. 60

In the following description, I have explained the method of making a cylinder having two concentric rings, the outer of which has been expanded more than the inner and consequently has a greater elastic 65 strength. The herein-described method is however applicable to the production of articles having more than two rings, and to those in which the ring having the highest elastic limit is placed in any desired position with relation to the other rings composing 70 the finished article. I believe my invention to be a broad one and therefore do not intend any limitations not expressly contained in the claim forming a part thereof. 75

The invention will be fully understood from the following description when taken in connection with the accompanying drawings, and the novel features thereof will be pointed out and clearly defined in the claim 80 at the close of this specification.

### In the drawings:

Fig. 1 shows the outer concentric member in process of being expanded.

Fig. 2 shows the outer concentric member 85 being annealed.

Fig. 3 shows the outer concentric member being assembled with an unexpanded inner member.

Fig. 4 shows the two members being ex- 90 panded.

Fig. 5 shows the annealing of the two members.

Fig. 6 shows the two members being again expanded. 95

Figs. 7 and 8 are diagrams illustrating the effects of the herein-described process.

### Referring now to the drawings:

At A is shown, what for convenience may be termed the outer concentric member, 100 which is of steel or a suitable alloy. In practicing my preferred method, this member is expanded by the apparatus described in my prior Patent No. 1,553,824, the expansion being carried to a point beyond the 105 elastic limit of the material and thereby increasing its elastic strength. The piece is preferably then annealed as described in my prior Patent No. 1,552,848, this being shown in Fig. 2. Next, a concentric inner 110

member B of an exterior diameter such that it will fit closely within the bore of member A is assembled with it. (See Fig. 3.) The two then are simultaneously expanded (see Fig. 4) as previously described, thereby raising the elastic limit of both members A and B. Thereafter (see Fig. 5), the whole is annealed and is again expanded. (See Fig. 6.) It will be understood that the expanding and annealing steps may be continued according to the final results desired.

The article in the condition shown may then be finished; if it is intended for use as a gun, it will be rifled.

The effects of the procedure already described will be best understood from an examination and comparison of the diagrams contained in Figs. 7 and 8. In Fig. 7 is shown a tube M having a thickness of one calibre. If it be assumed that this tube has been expanded in accordance with the method described in my prior Patent No. 1,553,824, and test-bars are cut from the metal to determine the elastic limit of the metal at different points along the radial line *a b*, it will be found that the elastic limit diminishes toward the exterior, as shown by the curve *d d*, which shows the elastic limits plotted against the distances radially. This decrease in elastic limit is due to the fact that the amount of increase in elastic limit resulting from cold working such as takes place when the tube is expanded is a function of the amount of flow of the metal, and since the metal on the outside of the tube flows less than that at the center, the increase in elastic limit is less. It results that the capacity of the metal on the outside of the tube to withstand expansion is not being used to the fullest possible extent.

In Fig. 8, I have shown a tube made up of two concentric members N and O, both of which have been expanded as previously explained. In this case the outer member

was expanded separately and the elastic limit of the material raised, as shown by the curve *g r* in dotted lines. The inner member was then inserted and the two members simultaneously expanded. The curve *e f* indicates the elastic limit of the inner member while the curve *g h* indicates that of the outer member after the final expansion. It will therefore be seen that the elastic strength of the outer member is considerably greater than that of the corresponding zone of the unitary tube shown in Fig. 7, and that of the finished tube as a whole is correspondingly greater. In other words, the elastic strengths of the outer layer of the outer member and of the inner layer of the inner member are not materially different and the former is equal to or greater than the latter.

As a consequence of these facts, the elastic limit of each section, except the inner one, is greater than the elastic limit of the corresponding zone of a unitary cylinder of identical size and composition, and the elastic strength of the composite tube as a whole is greater than that of a unitary tube of like size and composition due not only to increased elastic limit of the outer metal, but increased compression of metal at the bore. It will be understood, of course, that these figures are merely diagrams to make the effect more clear, and make no attempt to represent the conditions accurately.

What I claim is:

The method of making hollow articles which comprises expanding a hollow tubular member to increase its elastic limit, assembling therewithin a second tubular member and subjecting the latter to expansion until the elastic limit of its inner layer is not materially different from that of the outer layer of the first mentioned member.

In testimony whereof I affix my signature.

FREDERICK C. LANGENBERG.